

F. W. AYER.

## METHOD OF SEPARATING BARK FROM WOOD.

APPLICATION FILED MAY 23, 1910

979,914.

Patented Dec. 27, 1910.



*Witnesses:*

Josephine H. Ryan  
Charles D. Woodbury

Inventor:  
Med W. Ayer  
by Roberts, Roberts & Cushman  
Attest.

# UNITED STATES PATENT OFFICE.

FRED W. AYER, OF BANGOR, MAINE.

## METHOD OF SEPARATING BARK FROM WOOD.

979,914.

Specification of Letters Patent. Patented Dec. 27, 1910.

Application filed May 23, 1910. Serial No. 562,853.

*To all whom it may concern:*

Be it known that I, FRED W. AYER, a citizen of the United States, and resident of Bangor, in the county of Penobscot and State of Maine, have invented new and useful Improvements in Methods of Separating Bark from Wood, of which the following is a specification.

My invention relates to the preparation of wood for paper stock and consists of a process whereby the bark is effectively and economically removed from the wood without wasting any sensible portion of the wood fiber available for paper making.

While my process may be utilized for the separation of bark from wood to prepare the latter for the manufacture of stock for any grade of paper, it is particularly useful in cases where the stock is to be used in the manufacture of the higher grades of paper.

The preparation of wood pulp for paper making requires the elimination of the bark, for the reason that bark is peculiarly resistant to mechanical or chemical action.

Even small quantities of bark remaining adherent to wood will pass through all the pulp making processes and retain the form of fiber aggregations and a dark color; to some extent such bark particles find their way even into the finished paper product, producing blemishes therein known as "shives," which lower the value of the product. It is important, therefore, to the manufacture of any paper, and essential to

that of high grade paper, that wood bark shall be thoroughly eliminated from the stock. Thus, to be practically and commercially effective, any method of bark removal must be complete and perfect in its results.

This desideratum has been recognized from the earliest days of wood-pulp paper manufacture. In the beginning of this manufacture, bark was removed from the logs at the time of cutting, by means of a chisel-like tool called a "spud," and later, by hand shaving at the pulp mill. Subsequently, barking machines, employing a rotating disk with knives set radially in its face, were introduced, and are still extensively used for bark removal. These machines are hardly applicable to any material except the round logs, and even with such material, their operation is wasteful, because in order to reach the bark in hollows on the logs it is necessary

either to cut away a considerable part of the clear wood with the bark, or to resort to sub-

sequent hand shaving to remove the bark from these hollows.

Attempts to remove bark from slabs and edgings, which form the largest part of saw mill waste, with these rotary barking machines have not been successful or economical; it is dangerous to handle slabs and edgings in such machines, and the waste incident to cutting is so large that the expense of barking saw mill waste has been too large to justify its conversion into paper stock. Thus, slabs and edge strips from the saw mill have been of little value except as fuel, and even for this purpose their utility is limited, since their fuel value is not high enough to warrant shipment to any considerable distance, and because the large quantity of such waste usually exceeds the fuel demand at the mill where it is produced, and these slabs and edgings, which contain in the aggregate a large amount of wood fiber in itself perfectly adapted to paper manufacture, are for the most part burned in the open or left to rot. Moreover, the tops and branches of trees, which are now wasted altogether, contain in the aggregate large quantities of sound wood available for paper making purposes but for the fact that the difficulty presented by the adhering bark has heretofore prevented their use. It has also been proposed to strip the bark from sticks and logs by means of blades or strippers arranged in a rotary drum in which the logs are tumbled; but this method again has, in practice, met with only indifferent success for the reason that while there is less waste than by the cutting method, the process is not sufficiently thorough. Only those portions of the bark struck by the blades or strippers are removed and bark adhering to depressions or other irregularities in the stick or log escapes the strippers and has to be subsequently cut off by hand. Furthermore, this tumbling process is very slow, and the prolonged subjection of the wood to violent agitation and impact in the drum, results in splintered or "broomed" ends and edges of the wood which become filled with fine fragments of bark and other dirt which must be subsequently removed with difficulty or if not removed will deteriorate the quality of the paper stock.

My invention has for its object in general the amelioration of the above condition, the prevention of waste of good wood and the utilization of sticks, slabs, tops, branches

and other small pieces of wood which if successfully deprived of adhering bark, constitute good available wood fiber. The slabs and edge strips produced by the operation 5 of sawing a log into planks, are without further mechanical treatment in proper shape to be subjected to my improved process. Logs, sticks, tops or branches will preferably be scored split or sawed longitudinally 10 before being subjected to this process.

The preliminary effect of my process is the liquefaction of the bark cement so that it ceases to have an appreciable adhesive value, and the bark is ready to slip or fall 15 off the wood with very little mechanical effort applied to it. Pieces of bark of large extent, as on large slabs or full sized logs will, in this condition of the bark glue, adhere here by simple suction, or rather atmospheric pressure, so that more vigorous rubbing is required to remove such bark pieces than in the case of narrow edgings. Moreover, in order to provide a starting line for 20 the bark to come away from the wood, round logs should be slit or scored lengthwise, else 25 the unbroken ring of bark will by its own integrity, resist removal.

The process takes advantage of the fact that the bark of trees forms an integument 30 joined to the wood by cementitious or mucilaginous matter, and that the bark moreover is porous or spongy so that a solvent of the cement may readily penetrate the bark and reduce the cementitious material to a 35 condition resembling that of a solution in which its quality as an adhesive is temporarily, at least, destroyed. When the cement which secures the bark to the wood is thus softened, loosened, or reduced to solution, it 40 is quite easy by means of comparatively gentle mechanical processes, or even by hand, to remove the bark cleanly and completely from the wood. To this end, I immerse the wood, 45 from which the bark is to be removed, in water, at or approximating the boiling point, keeping the wood wholly submerged for a sufficient period of time for the hot water to penetrate the bark and dissolve the soluble cementitious or mucilaginous material which 50 holds the bark to the wood. By experiments, chiefly with spruce sticks, consisting of slabs and edgings taken directly from the saw mill I have found that by immersing the wood for about 35 minutes in water at a 55 temperature of from 180° F. to 212° F., the cementitious matter holding the bark to the wood will be dissolved, and the bark will become so loosened from the wood as to separate of itself, or require only a comparatively 60 gentle mechanical treatment such as attrition caused by making the pieces of wood slide over each other, to remove it.

The bark in its natural state is of a somewhat porous and spongy structure and tends 65 to imbibe the water and admit it to the cem-

entitious matter which binds the bark to the wood. This cementitious matter however is not readily soluble in cold water, or in water substantially below the temperatures mentioned, and if soluble at all below such temperatures, it would require a treatment of such long duration—many months in fact—as to be impracticable as a decorticating process. I have discovered however that said cementitious matter is very readily 70 and rapidly soluble in water at temperatures above about 180° F. and the treatment aforesaid in such hot water has two effects: It dissolves the intercellular cementitious matter in the bark itself, which binds the bark 75 fibers together and is of the same or similar character to that which binds the bark to the wood, thus opening the bark to the free and rapid penetration of the hot water therethrough; and upon reaching the cementitious 80 matter between the bark and the wood it dissolves that and renders the bark easily 85 removable.

At the end of the hot water treatment, if the bark has not separated of itself, it should 90 be stripped or knocked off at once while the wood is wet, otherwise the residual cementitious matter in solution between the bark and the wood, will upon drying, again cement the bark to the wood. I therefore subject the sticks to a mechanical stripping treatment after the action of the hot water and while the cementitious matter is still in solution and hot, to knock or otherwise separate the bark from the wood, which now 95 only adheres by reason of the suction between the two close fitting wet surfaces.

The above described treatment of split tops, branches, edges and slabs, involves immersion of the bark-carrying wood pieces 100 in an abundance of hot water, which impregnates the wood and bark, and supplies enough water, remaining in and upon the pieces, to hold the cementitious matter in solution for a time amply sufficient to allow 105 for mechanical removal of the bark which remains loosely adhering to the wood, after the latter has been taken from the hot water.

In the accompanying drawings is illustrated 110 an apparatus appropriate for performing my new process. This apparatus is the joint invention of myself and others and constitutes the subject of a separate application to be filed simultaneously herewith, jointly by myself and others.

Figure 1 of said drawings represents a 115 vertical, longitudinal, central section, partly broken away, of an apparatus for removing bark from wood; and Fig. 2 represents a longitudinal section on broken lines 2—2 120 125 of Fig. 1.

A represents a long and relatively narrow and shallow tank for holding the water, which is heated by steam introduced through jets *b*, *b*, leading from the steam 130

pipe B which is connected with any suitable source of steam supply.

6 C is a belt or apron, mounted to move slowly in the direction of the arrows, the lower stretch of the belt C being just submerged in the water in tank A.

The wood W is fed into the intake end of the apparatus, which is the right hand end as viewed in the drawings, and is carried 10 slowly to the outlet end, which is the left hand end as viewed in the drawings, whence it is discharged with the stream of water, upon the chute or incline D. Water is continuously introduced through pipe P at the 15 intake end of the tank, so that there is a continuous flow of water through the tank from the intake end to the outlet end, and the belt C is timed to move at substantially the same speed as the stream of water, the belt and 20 stream of water thus carrying the wood forward, and the belt holding it at all times submerged. The length of the tank and the rate of the supply and overflow of the water are so proportioned that the submerged 25 wood sticks occupy about 35 minutes in traveling from end to end of the tank.

The chute D is provided with projections preferably arranged staggered or irregularly, as shown, and tumbles the wood about 30 as it falls down the chute, thus knocking off the bark which has become "unglued" in the hot water bath. The wood and the separated bark pass down the chute D by gravity, assisted by the overflow stream of water, 35 upon a sloping platform E formed of spaced slats. The water and smaller pieces of bark pass through the platform E into a tank T while the wood sticks, entirely cleaned of the bark, and the larger pieces of bark which 40 cannot pass between the slats of the platform E, slide down platform E into a conveyer F, which carries the material away.

Within the tank T is a screen S to strain 45 out the bark and the water is taken from tank T by pipe p and pump p' to the inlet pipe P, thus maintaining a continuous circulation of the hot water through the apparatus with comparatively little waste of heat.

50 Said apparatus is herein described merely to illustrate one suitable method of practicing my process, but it will be understood that my process may be performed by other suitable means.

55 The practical result of the above described process, as demonstrated upon a commercial scale, is the saving of from 20% and upward of the sound wood fiber of which the logs and sticks are composed and which has 60 heretofore been wasted, practically increasing the forest yield by that considerable proportion. The percentage saved varies according to the size, and to some extent, the shape of the logs themselves, and also depends upon the amount of available wood 65

fiber reclaimed by this process from tops and branches heretofore wasted.

The effect of the abundance of hot water on the bark-cement is herein expressed by the term "solution." I use that, and associated terms of description not in a strict sense; I understand that the effect of water on such mucilaginous matter is not exactly to dissolve it, but to swell and liquefy it, rendering it more and more attenuated, and 70 less adhesive, as the proportion of water, or "solvent," increases.

To derive full utility from the above described process, after the bark glue has become thoroughly liquefied by steeping in an 80 abundance of hot water, the scored logs, sticks, slabs, edgings, etc., should forthwith, that is to say, before the water contained in and carried by them has a chance to become 85 cold or evaporate, be subjected to such gentle mechanical treatment as will peel or rub off the loosened bark. While this may be done easily by hand, an automatic mechanical treatment is preferable for reasons of economy. All that is necessary is to cause 90 the wood pieces to slide and rub over each other, the bark covering each piece will then come off, usually as a single strip, leaving the wood clean and bare, stripped of bark even in the depressions. Preferably the 95 bark-stripping is done after the wood pieces are removed from the steeping bath; attrition between the pieces while immersed in water, while reasonably effective, is not so economical, since the flotation and lubricant 100 effect of the water to a degree interferes with the effective rubbing of one piece on another. The reduction of the bark-cement by this method brings to bear two effective agents, 105 heat and an abundance of water, as distinguished from the heat alone which might be furnished by steam, or moisture alone as would be supplied by water at ordinary or even warm temperatures. For practical 110 purposes a minimum temperature of 120° Fahrenheit is requisite, the preferred temperatures lie between 180° Fahrenheit and boiling point.

I claim:

1. The method of loosening bark from 115 wood which consists in immersing pieces of wood with bark attached in an abundance of water in liquid as distinguished from vaporous condition, at a minimum temperature of 120° Fahrenheit for such time as 120 suffices to so far liquefy all the cementitious matter binding the bark to the wood that it loses its character as an effective adhesive, and so that the wood and bark are impregnated with sufficient water to hold 125 said cementitious matter in liquefied condition for a considerable time.

2. The method of loosening bark from 130 wood which consists in immersing pieces of wood with bark attached in an abundance

of water in liquid as distinguished from vaporous condition, at a minimum temperature of 120° Fahrenheit for such time as suffices to so far liquefy all the cementitious matter binding the bark to the wood that it loses its character as an effective adhesive, and so that the wood and bark are impregnated with sufficient water to hold said cementitious matter in liquefied condition for a considerable time, then removing the pieces of wood from the water and subjecting them to mutual attrition while the cementitious matter is still thus liquefied.

3. The method of separating bark from wood which consists in severing the bark covering of pieces of wood along the grain, immersing the wood thus prepared in an abundance of water in liquid as distinguished from vaporous condition, at a minimum temperature of 120° Fahrenheit for such time as suffices to so far liquefy all the cementitious matter binding the bark to the wood that it loses its character as an effective adhesive and so that the wood and bark are impregnated with sufficient water to hold said cementitious matter in liquefied condition for a considerable time.

4. The method of denuding wood of its bark to make it suitable for paper pulp which consists in steeping the bark covered wood by immersion in an abundance of water at a minimum temperature of 120° Fahrenheit thereby liquefying all the cementitious matter between the bark and the

wood and impregnating the wood and bark with sufficient water to hold said cementitious matter in such liquefied condition as renders the bark capable of removal from the wood in its entirety by the aid of gentle mechanical treatment such as the attrition of one piece of wood upon another, and subsequently, while the cementitious matter is still liquefied, subjecting the pieces of wood to such mechanical treatment.

5. The method of denuding wood of its bark to make it suitable for paper pulp which consists in steeping the bark covered wood by immersion in an abundance of water at a temperature between 180° Fahrenheit and boiling point, thereby liquefying all the cementitious matter between the bark and the wood and impregnating the wood and bark with sufficient water to hold said cementitious matter in such liquefied condition as renders the bark capable of removal from the wood in its entirety by the aid of gentle mechanical treatment such as the attrition of one piece of wood upon another, and subsequently, while the cementitious matter is still liquefied, subjecting the pieces of wood to such mechanical treatment.

Signed by me at Bangor, Maine, this twentieth day of May, 1910.

FRED W. AYER.

Witnesses:

JOHN C. WILSON,  
FRED R. AYER.